

E. E. NOVOTNY.

SOUND RECORD.

APPLICATION FILED JULY 21, 1920. RENEWED MAY 3, 1921.

1,398,145.

Patented Nov. 22, 1921.

*Fig. 1.*



*Fig. 2.*



*Fig. 3*



INVENTOR

Emil E. Novotny

BY

Meyers, Cavanagh & Hyde.  
his ATTORNEYS

# UNITED STATES PATENT OFFICE.

EMIL E. NOVOTNY, OF LOGAN, PHILADELPHIA, PENNSYLVANIA, ASSIGNOR TO JOHN STOGDELL STOKES, OF PHILADELPHIA, PENNSYLVANIA.

## SOUND-RECORD.

1,398,145.

Specification of Letters Patent. Patented Nov. 22, 1921.

Application filed July 21, 1920, Serial No. 397,927. Renewed May 3, 1921. Serial No. 466,535.

To all whom it may concern:

Be it known that I, EMIL E. NOVOTNY, a citizen of the United States, and resident of Logan, Philadelphia, in the county of Philadelphia and State of Pennsylvania, have invented certain new and useful Improvements in Sound-Records, of which the following is a specification.

This invention relates to the manufacture of sound records, such as are used in connection with phonographs and similar machines.

In the present instance it is my purpose to provide an exceedingly thin, light record of great strength and durability which may be manufactured and marketed in vast quantities at a minimum expense, thereby rendering it particularly adapted for the reproduction of popular music, speeches, lectures and the like. Furthermore, due to its lightness and lack of bulk this record will occupy but very little space in shipping and filing, and may be sent through the mails, or by express at a relatively low cost when compared with the ordinary record. Furthermore, owing to the peculiar physical characteristics of my record it is practically unbreakable and therefore the loss incident to the destruction of the ordinary brittle records in packing, transportation, and actual usage is practically eliminated.

With the above recited object and others of a similar nature in view my invention consists in the construction, combination and arrangement of parts set forth in and falling within the scope of the appended claims.

In the accompanying drawings:

Figure 1, is a cross sectional view illustrating the various layers or strata of material which are employed in the manufacturing of my preferred form of sound record.

Fig. 2, is a cross sectional view of a complete preferred form of sound record,

Fig. 3, is a plan view on a reduced scale of the intermediate or reinforcing plate which is embodied in the record shown in Fig. 2,

Fig. 4, is a similar view of a modified form of reinforcing plate.

Referring now to the accompanying drawings in detail, the letter A indicates an intermediate or central reinforcing plate, which is preferably composed of metal, such as a very thin flexible sheet of lead, tin, steel,

aluminum or the like, this plate being preferably of a thickness of approximately one one thousandth of an inch. In Fig. 3 I have shown this plate A as in the nature of a solid sheet, with the exception, of course, of the central spindle opening, and in Fig. 4 wherein a modified form of the plate is exhibited it will be noted that it is in the nature of a perforated or open mesh sheet, designated at A'. This reinforcing plate A, which in its preferred form is substantially solid or imperforate, is, in the manufacture of the record coated upon both faces with cement as shown at B, for the purpose of causing the adherence of other layers and strata as hereinafter described. This cement may be of a suitable character for the purpose and I have found a good adhesive to be a composition of a phenol and aldehyde condensation product mixed with barium sulfate, and the whole reduced by the use of a suitable solvent such as alcohol to a varnish-like consistency. Of course, instead of using this particular condensation product cement I may employ any means for securing the other layers or strata to this central reinforcing plate. To each side of the cement-coated reinforcing plate I apply a sheet of material shown at C. The sheets C are preferably composed of a fibrous material, such as a thin layer of straw board, chip board or the like, impregnated, but not fully saturated, with a condensation product formed from phenol and an aldehyde, and which as is well known is capable of reacting and hardening and setting under heat and pressure. There are a number of such condensation products on the market, some commercial forms being known as bakelite and condensite, and these are well adapted for my purpose. I do not fully saturate the fiber sheets, because I want to avoid the possibility of the fluid-like condensation product oozing or flowing out of the fiber during the impression period, as when the record is being molded. The fiber sheets may be so impregnated by dipping the same in a bath of the liquid or fluid of phenolic condensation product which is about the consistency of a thin varnish. After the fiber sheets have been so dipped they may be dried in an oven to drive off the solvent, and to cause a partial reaction of the condensation product, causing the same to partly harden and set, but not to a complete

final form. After the fiber impregnated sheets have been thus dried out they are attached to the central reinforcing plate A by the cement shown at B and as above described. In order to insure the proper adherence of the fiber impregnated sheets C to the central reinforcing plate, after they have been applied, the sheets thus assembled may be placed in a press and sufficient pressure exerted to cause the uniform and adequate union of the fiber sheets to the central plate. The outer face of each impregnated sheet C is then provided with a layer or coating, indicated at D. These intermediate layers or coatings D may be, for the sake of convenience termed barrier coats, and act to prevent the absorption of tones, particularly over-tones and under-tones by the fiber sheets C, during the playing of a selection, and thereby insure full, clear and resonant tones. These coatings D also act to prevent the penetration of the material of the exterior or face coatings E into the body of the fiber sheets C. Both the intermediate coatings D and the exterior coatings E are composed of a cementitious material, such as a synthetic resin in the nature of a condensation product formed by the reaction of a phenol and an aldehyde, and the commercial products bakelite and condensite heretofore mentioned may be used for this purpose. However, it is desirable that the intermediate coatings be made much harder and denser, and more compact than the exterior coatings E, and consequently in preparing the cementitious material for the intermediate coatings D I mix therewith barium sulfate, preferably in proportion of one part of barium sulfate to two parts of phenolic gum. Of course, when the coatings are applied the cementitious material is of a varnish-like nature, and will subsequently harden and set under heat and pressure as is well known. The barium sulfate will harden the cementitious material of the intermediate coatings D to such an extent that the layers will be exceedingly dense and compact. The intermediate coatings D are applied by dipping the article into a bath of the synthetic resinous varnish, and after a relatively thin coating has thus been received by the article it may be placed in an oven and subjected to a degree of heat, say, two hundred to three hundred degrees F., for a sufficient length of time, say from ten to sixty minutes, for the purpose of drying the coatings by driving off the solvent, and at the same time partially hardening and setting the coatings, but not to final infusible form. Subsequently the article at this stage of its manufacture may now be dipped in another bath of cementitious material, such as a synthetic resin heretofore mentioned, but of a richer mixture than is used for the intermediate coatings D, and which richer

mixture lacks the barium sulfate or hardening agent, a quantity of filler, such as lamp black being mixed with the phenolic varnish which is to form the outer coatings E. The article is then again placed in an oven and heated at from two hundred to three hundred degrees F., for from ten to sixty minutes to dry out the coatings E and to partially harden and set the same to a non-flowing condition, but at this stage the coatings are still capable of taking molding impressions. It is to be understood that the fiber sheets C and the coatings D and E are exceedingly thin, for example, each fiber sheet may be of a thickness of about eight one thousandths of an inch, the intermediate coatings D may be of a thickness of one one thousandth of an inch and the exterior coatings E may be of a thickness of two one thousandths of an inch. The blank thus prepared may now be placed in contact with the ordinary record matrix and subjected to heat and pressure against the same for a sufficient length of time, say for about one to five minutes, to mold the sound grooves shown at F in the faces of the record blank, and at the same time cause the hardening and setting of the synthetic resinous material to its final form.

The result will be a sound record which is exceedingly thin and light, and which possesses a certain degree of flexibility, so that, in some instances as where a thin, lead sheet is used for reinforcement, the record may be rolled and shipped in a tube or cylinder, if desired. The record will maintain its flat form however under weather conditions, as the possibility of warping is eliminated due to the thinness of the coatings and the metallic reinforcement. In the complete record the outer coatings E will be found to be of a thin, skin-like nature possessing greater tensile strength than the intermediate coating, but not so hard.

Such a record is not subject to breakage under shocks and jars as is the case with ordinary, brittle records, nor will the sound grooves thereof be abraded or cut down by a steel needle to the same extent as grooves in an ordinary record, this being due to the tough, tenacious, skin-like character of the exterior coatings or layers E.

If desired, the cementitious or synthetic resinous material contained in the blank, may be hardened to such an extent, prior to the molding of the record itself, that little or no further reaction will be required at the time of molding to reduce the blank to its final hard and set form. By so pre-hardening the blank it only requires heating for a short time during the molding against the sound matrix to enable the necessary impression to be made and the hardening and setting of the blank completed. Consequently the time actually required for mold-

ing the record against the matrix may be greatly shortened, and indeed the record after molding may then be readily stripped from the matrix while in a heated or partially heated condition, thus releasing the matrix for the molding of another blank. Consequently the output of a matrix may be greatly increased.

As above stated in Fig. 4 I have shown at A' a modified form of reinforcing plate, in this instance the plate being of a reticulated nature or provided with perforations or openings. This will enable the production of a slightly lighter record, and at the same time during compression the material may flow through the openings and tend to more firmly unite or anchor the reinforcing plate in the center of the record.

While I have herein shown and described certain preferred embodiments of my invention I wish it to be understood that I do not limit myself to all the precise details set forth by way of illustration, as modification and variation may be made without departing from the spirit of the invention or exceeding the scope of the appended claims.

What I claim is:

1. A sound record comprising a metallic

reinforcing member, a fiber sheet impregnated with a hard and set synthetic resin 30 united with said member, and a grooved face section with a hard and set synthetic resin imposed upon the fibrous sheet.

2. A sound record comprising a central reinforcing plate, a fibrous sheet united with 35 said plate, a relatively hard layer of synthetic resin imposed upon the fibrous sheet, and a relatively soft coating of synthetic resin imposed upon the relatively hard layer, said relatively soft layer having sound 40 grooves formed therein.

3. A sound record comprising a central reinforcing plate, fibrous sheets united with opposite sides of the reinforcing plate, said sheets having hard and set synthetic resin 45 incorporated therein, barrier layers of relatively hard synthetic resin imposed upon the fibrous sheets, and exterior coatings of relatively soft synthetic resin imposed upon the barrier layers and having sound grooves 50 formed therein.

Signed at New York city, in the county of New York, and State of New York, this 15th day of July, A. D. 1920.

EMIL E. NOVOTNY.